# EUROPEAN PATENT SPECIFICATION

(11) **EP 0 686 229 B1**
(45) Date of publication and mention of the grant of the patent: **26.03.1997**
(21) Application number: 94907629.3
(22) Date of filing: 25.02.1994
(51) Int. Cl.: F01D 5/20

(54) **METHOD OF PRODUCING AN ABRASIVE TIP ON A TURBINE BLADE**
METHODE ZUR AUFBRINGUNG EINER ABRASIVEN SCHICHT AUF DAS ENDE EINER TURBINENSCHAUFEL
PROCEDE DE PRODUCTION D'UNE POINTE ABRASIVE SUR UNE AUBE DE TURBINE

(30) Priority: 25.02.1993 GB 9303853
(43) Date of publication of application: 13.12.1995
(73) Proprietor: Praxair S.T. Technology, Inc., North Haven, CT 06473 (US)
(72) Inventor: FOSTER, John, Weston-super-Mare, Avon BS22 9QD (GB); TAYLOR, Alan, Weston-super-Mare, Avon BS22 0QE (GB); CHATTERLEY, Martin Patrick, Weston-super-Mare, Avon BS22 9AG (GB)
(74) Representative: Robinson, Anthony John Metcalf
(86) International application number: GB9400374
(87) International publication number: WO9419583

(56) References cited:
- EP-A- 0 355 051
- EP-A- 0 404 020
- FR-A- 2 649 125
- GB-A- 2 162 201
- GB-A- 2 167 446
- GB-A- 2 182 055
- GB-A- 2 241 506
- US-A- 4 345 977
- US-A- 4 584 081

## Description

This invention relates to blades for turbines and compressors and in particular relates to the production of blade tip seals.

It is known to provide at the tip of a gas turbine blade a tip portion comprising abrasive particles which are embedded in a matrix, the tip being intended to run against the surface of a shroud of a material which is softer than the abrasive particles. By this means, it is possible to produce, by the abrasive action of the particles on the shroud, a gap between the tip and the shroud which is very small, thus minimising gas losses. In one particular example where this technique is used, the matrix comprises a major part of cobalt and minor parts of chromium, tantalum and alumina while the lining material of the shroud comprises a major part of cobalt with minor parts of nickel, chromium and aluminium and a small quantity of yttrium. Various methods for producing such tips have been proposed. In one example, detonation spray coating of the matrix is used. In another example there is first produced an inner tip portion of mainly nickel and cobalt with additional ingredients by casting as a single crystal and the inner tip portion is, after shaping, diffusion bonded to the tip of the blade body. The abrasive portion of the tip is then formed on the inner tip portion by electrodeposition of alternating layers of chromium and nickel about the abrasive particles. The outer tip portion can then be aluminided to produce a matrix alloy of NiCrAl.

There has been described in GB-A-2241506 a method of producing a gas turbine blade having an abrasive tip which comprises producing a binding coat on the tip of the blade body by electrodeposition, the binding coat comprising MCrAlY where M is one or more of iron, nickel and cobalt, anchoring to the binding coat coarse particles of an abrasive material by composite electrodeposition from a bath of plating solution having the abrasive particles suspended therein, and then plating an infill around the abrasive particles. It has been found that this method, all stages of which are of a metal plating nature and are therefore relatively inexpensive and readily controllable, produces a very effective abrasive blade tip.

All the methods for producing blades with tip seals are expensive and time consuming and it is an object of the present invention to provide a method of producing blades with tip seals which is cheaper and more satisfactory than the prior methods referred to.

According to the present invention, compressor or turbine rotor blades are assembled on a compressor or rotor disc and abrasive tips are produced on the tips of the assembled blades by electrodeposition or by electroless deposition.

Production of the tips on the assembled blades has several advantages, the chief of which is that it is possible to carry out various production steps on the assembled disc without subsequent disassembly. The present practise is for the blades to be assembled on the disc and for the blade tips to be machined to produce a properly balanced disc. The blades are then marked, disassembled from the disc, mounted on a jig, tipped, removed from the jig and then reassembled on the disc in the same order and positions that they previously occupied. By proceeding in accordance with the invention, one of the two assembly operations, jigging and dejigging, the marking and the disassembly are avoided and unbalancing due to the blades being reassembled in slightly different attitudes or positions from those previously adopted is obviated.

The process according to the invention is particularly suited to blade tipping using the methods described in GB-A-2241506 in which a binding coat is produced on the tip of each blade by electrodeposition, coarse particles of an abrasive material are anchored to be binding coat by composite electrodeposition of the particles and an anchoring coat and then plating an infill around the particles. The binding coat may comprise MCrAlY where M is one or more of iron, nickel and cobalt. The anchoring coat may be of cobalt or nickel or MCrAlY as defined above and the infill may also be MCrAlY and defined above.

The blades are tipped while assembled on a compressor or rotor disc, which term is intended to cover bosses, rings and similar blade mounting elements which terms are used for substantially the same structures. Although it is possible to treat the discs individually, further benefits can be obtained by first assembling a plurality of rings together to form a part or a whole turbine or compressor rotor. This again reduces the steps required and helps to maintain balance.

Various particles may be employed. Examples include zirconia, alumina and various nitrides, silicides and borides known from the abrasive art. The preferred abrasive is cubic boron nitride, preferably having a particle size between 125 and 150 µm. It is possible for the infill, or at least the upper or outer portion thereof, to include abrasive particles of a size substantially smaller than the main abrasive particles, for example approximately 20 µm.

The MCrAlY of the binding coat, the anchoring layer where this is MCrAlY, and the infill where this is MCrAlY may have various compositions of which suitable examples are described in British Patent Specification GB-2167446B. The electrodeposition may be effected by various forms of apparatus. However, suitable forms of apparatus are described in British Patent Specification Nos. GB-2182055A and European Patent Specification No. EP-0355051A. These describe apparatus which comprises an electroplating tank which is divided into two zones by a vertical wall extending from close to the bottom of the tank up to just beneath the surface of the solution in the bath. Gas is admitted to one of the zones to induce an upward flow of solution therein, the solution, with particles entrained therein, spilling over the weir formed by the upper edge of the division wall and descending in the second zone in which the article to be coated is located. The latter specification describes rotating the article with a stop-start or quick-slow cycle.

Where the infill is of MCrAlY, that is it consists of particles of CrAlY in a metal matrix, the deposition of the infill is preferably accompanied by vibration of the assembly, preferably in a vertical direction. It is believed that such vibration ensures an even distribution of CrAlY particles, particularly in those regions which are shaded by the overhang of the abrasive particles and which regions might otherwise be depleted of particles. The frequency of the vibration is preferably between 10 Hz and 1 kHz, the particularly preferred figure being about 50 Hz. A peak acceleration of up to 10 g is preferred. It is believed that a particularly good result is achieved by vibrating at two alternating levels, for example a vibration with a peak level of about 2 g alternating with a vibration with a peak level of about 10 g. Preferably, each lower level phase is longer than each higher level phase; thus the lower level phases may be for between 30 seconds and 2 minutes duration with a peak acceleration of about 2 g and the higher level phases may be for about 5 seconds duration with a peak acceleration of about 10 g.

The invention may be carried into practice in various ways but a process of producing a gas turbine blade in accordance with the invention together with apparatus suitable for carrying out the process will now be described by way of example with reference to the accompanying drawings in which:
Figure 1 is a perspective view of one of the plating baths used in the process;
Figure 2 is a side elevation of the apparatus shown in Figure 1;
Figure 3 is a front elevation of the apparatus shown in Figure 1;
Figure 4 is a perspective view of a fixture used in the apparatus shown in Figures 1 to 3;
Figure 5 is a front view of the fixture shown in Figure 4 with an assembly mounted thereon; and
Figure 6 is an enlarged section through part of the tip region of a blade having an abrasive tip produced in the manner to be described.

The process to be described is intended to form abasive tips on the blades of a as turbine rotor assembly 52 which is shown in Figure 5. The assembly comprises five turbine discs 53 mounted on a hollow shaft assembly 54 forming part of the complete turbine. The shaft assembly is mounted on a shaft 26 for the tipping process which will be described below. Each of the discs 53 has mountings, for example fir-tree slots, in which the roots of the blades are mounted. It should be emphasised that in the preferred procedure the blades are mounted in the discs in their final positions and will not subsequently be disassembled from the discs.

The tipping process is carried out in the apparatus shown in Figures 1 to 3 of the drawings. This comprises a vessel or container 1 having a parallelepiped shaped upper portion 2 and a downwardly tapering lower portion 3 in the form of an inverted pyramid which is skewed so that one side face 4 forms a continuation of one side face 5 of the upper portion.

The vessel 1 contains a partition 6 which lies in a vertical plane parallel to the side faces 4 and 5 of the vessel and makes contact at its side edges 7 and 8 with the adjacent vertical and sloping faces of the vessel. The partition thus divides the vessel into a larger working zone 9 and a smaller return zone 11. At its bottom the partition 6 terminates at a horizontal edge 12 above the bottom of the vessel to afford an interconnection 13 between the working zone 9 and the return zone 11. At its top, the partition 6 terminates at a horizontal edge 14 below the top edges of the vessel 1.

At the bottom of the return zone 11 there is an air inlet 15 which is connected to an air pump (not shown). Mounted in the working zone 9 is a fixture 21 to which the assembly to be coated is mounted, the fixture 21 being arranged to position the assembly within the vessel in a manner to be described in greater detail below. Conductors, not shown, are provided to apply a voltage to the assembly mounted on the fixture 21 relative to an anode which is suspended in the working zone.

To use the apparatus to codeposit a coating on the blade tips of the assembly, the assembly is mounted on the fixture 21 which is positioned in the vessel as shown. Before or after the positioning of the fixture, the vessel is filled to a level 17 above the top edge 14 of the partition 6 with a plating solution containing particles to be co-deposited. Air is admitted to the inlet 15 and this rises up and the return zone 11, raising solution and entrained particles. At the top of the return zone. The air escapes and the solution and particles flow over the broad crested weir formed by the top edge 14 of the partition and flow down past the assembly on the fixture 21. At the bottom of the working zone 9, the particles tend to settle and slide down the inclined sides of the vessel towards the interconnection 13 where they are again entrained in the solution and carried round again.

As the downwardly travelling particles in the working zone 9 encounter the tips of the blades at the top of the assembly, they tend to settle on the these tips where they become embedded in the metal which is being simultaneously plated out.

The fixture 21 on which the workpieces to be coated are mounted is shown in detail in Figures 4 and 5, in simplified form in Figures 2 and 3 and is omitted from Figure 1 for reasons of clarity. The fixture 21 comprises a deck 22 which fits over the top of the vessel 1, a depending pillar 23 towards one end and a depending pillar 24 at the other end, the pillars having journals 25 in which the ends of the shaft 26 of the assembly are mounted. The deck 22 supports an electric motor 31 which rotates the shaft 26 through a vertical shaft 32, a first bevel gear 33 and a second bevel gear 34 mounted on a spindle 35.

At each end of the underside of the deck 22 there are springs 41 by which the jig is supported on the edges of the vessel 1 as seen in Figures 2 and 3. Mounted on the deck 22 is a vibrator 42 whose operation can be adjusted as required by a controller, not shown. An electronic motor controller 43 is mounted on the deck 22 and is connected by lines 45 to the motor 31. The controller 43 is designed so that the motor 31 is driven in one direction only so as to rotate the shaft 26 about a horizontal axis.

The use of apparatus of the construction described to produce abrasive tips on the gas turbine blades will now be described.

The assembly 52 is degreased in a vapour degreaser or a proprietary degreasing agent such as GENKLENE (Registered Trade Mark). The assembly is then grit blasted as necessary to provide a key for the masking wax and the assembly is then inserted into a wax bath to mask all the surfaces of the discs and blades. The assembly is then mounted in journals and rotated so that the tips of the blades move past a wiper which removes the masking wax from the tips of the blades. The assembly is then given an anodic clean for five minutes at 6 to 8 volts in a cleaning solution consisting of sodium hydroxide/gluconate/thiocyanate and is then rinsed thoroughly in cold running water. The exposed tips of the blades are then etched by submerging the assembly in a solution comprising approximately 300 gms/1 ferric chloride, 58 gms/1 hydrochloric acid and 1% hydrofluoric acid (60% w/w) for five minutes at room temperature and again rinsed thoroughly in cold running water. The assembly is then placed in a nickel chloride bath to provide a strike which is given at 3.87 amps per square decimeter (36 amps per quare foot) for four minutes. The strike bath comprises approximately 350 gms/1 nickel chloride and 33 gms/1 hydrochloric acid.

The assembly is then placed in the fixture shown in Figure 4 and the fixture is placed in the apparatus shown in Figures 1 to 3. The bath contains a cobalt plating solution with 20 to 30 weight percent particles of CrAlY containing 67-68 parts by weight Cr, 29-31 parts by weight Al and 1.5 to 2.4 parts by weight Y with a size distribution both in the bath and in the as-deposited coating as given in the following table, the columns relating to the size band being the upper and lower limits of the cut measured in micrometers.

**Table**

| Size Band | | Per Cent |
|---|---|---|
| 118.4 | 54.9 | 0 |
| 54.9 | 33.7 | 0 |
| 33.7 | 23.7 | 0.3 |
| 23.7 | 17.7 | 1.3 |
| 17.7 | 13.6 | 4.3 |
| 13.6 | 10.5 | 17.7 |
| 10.5 | 8.2 | 38.1 |
| 8.2 | 6.4 | 18.3 |
| 6.4 | 5.0 | 12.3 |
| 5.0 | 3.9 | 8.2 |
| 3.9 | 3.0 | 0.1 |
| 3.0 | 2.4 | 0 |
| 2.4 | 1.9 | |

Plating is continued for a period of 4 hours at a current density of 0.075 amps per decimeter (10 amps per square foot) with the controller set to rotate the motor at such a speed as to rotate the assembly at 0.33 revolutions per minute. Air is admitted continuously to maintain circulation of the solution and suspended CrAlY particles. This plating provides a binding coat of CoCrAlY on the tips of the blades to a thickness of between 25 and 50 µm. Deposition of CoCrAlY from the bath described will produce a layer having a composition which is approximately in weight percent: Al 10, Cr32, Y 0.5 and the balance Co.

The assembly is then rinsed over the tank with demineralised water and then removed from the region of the tank and rinsed in running water. The holder is then placed in a Woods nickel bath or 1 volume percent sulphuric acid bath to reactivate the surfaces and the assembly is then placed in a second bath similar to the first bath except that in place of the CrAlY particles it contains particles of cubic boron nitride of 100/220 mesh i.e. approximately 125-150 µm. Initially, no air is admitted through the inlet and plating is commenced at 2.7 amps per decimeter (25 amps per square foot) and then air is switched on for a period of 5 seconds. The boron nitride particles go into circulation and cascade over the assembly. Plating is then continued without the admissions of air for a period of approximately 40 minutes to secure the particles resting on the blade tips to the tips. It may be found that in some cases it is beneficial to have a further burst of 5 seconds of air after 20 minutes to ensure a uniform and maximum distribution of CBN particles over the blade tip surfaces.

The assembly is now removed from the CBN bath, is rinsed over the tank and is then rinsed in a static bath and finally rinsed thoroughly in running water. The surfaces being coated are then reactivated in a Woods nickel or 1% sulphuric acid bath and the fixture is replaced in the CoCrAlY bath. The motor is activated to rotate the assembly at 0.33 rpm and plating is continued for 7 hours at 1.075 amps per decimeter (10 amps per square foot) with continuous admission of air to maintain circulation of the solution and suspended CrAlY particles. This fills the spaces under and around the CBN particles with CoCrAly to a depth which, as can be seen in Figure 6, leaves the tips of the abrasive particles slightly proud of the surrounding CoCrAly.

During the infilling process, the provide a matrix around the particles, the assembly may be rotated with a start-stop action. Thus the motor is controlled to produce a rotation of the assembly unidirectionally and at a speed of one rotation in 3 minutes with the rotation being intermittent with 10 second stop periods being interspersed with three second go periods. Optionally in addition the vibrator may be used. The vibrator is arranged to give a vibration at a frequency of 50 Hz with alternating periods of high intensity and low intensity vibration, the high intensity periods having a duration of 5 seconds and a peak acceleration of 10 g and the low intensity periods having a duration of 75 seconds with a peak acceleration of 2 g. The vibration and the rotation produce homogeneous infill and ensure that the CrAlY particles reach the areas shadowed by the CBN particles.

At the end of the infill stage the fixture is removed and the assembly is rinsed over the tank with demineralised water and then rinsed thoroughly in running water. The masking material is then removed and the assembly is taken out of the jig and degreased. After inspection the assembly is then heat treated from between 1/2 and 1 hour at 1090 plus or minus 10°C in vacuum or in 50-100 millibar partial pressure argon and fast gas quenched. The blades may then be aluminized by one of the well-known processes such as pack aluminizing.

One of the tips produced in the manner described is shown in section in Figure 6 and can be seen to comprise the body 80 of the blade, a binding coat 81 of MCrAlY of a thickness, in this example, of 25-50 µm, an anchoring coat 82 of MCrAlY of a thickness of 10-20 µm in which is anchored the bottom portions of the abrasive particles 83 of cubic boron nitride with a particle size of 125-150 µm, and an infill 84 of MCrAly with a thickness of 70-110 µm.

It will be understood that the tips shown in Figure 6 are not identical to those produced as specifically described above; since the second bath mentioned above is said to be similar to the first Cobalt and CrALY plating bath except that in place of the CrALY it contains CBN particles, the anchoring coat in the specific process described is Co, not CoCrALY. As mentioned previously in this specification, the anchoring coat may be of Co, Ni or MCrALY as defined above.

Instead of particles of pure cubic boron nitride it would be possible to use particles of this or another abrasive which are coated with a material which will protect them, for a time at least, from severe oxidation. For example, it would be possible to use cubic boron nitride particles which had been given a substantially air-impermeable coating of aluminium oxide or an intermetallic such as nickel aluminide.

## Claims

1. A method of producing abrasive tips on compressor or turbine rotor blades by electrolytic or electroless deposition, characterised in that at least part of the deposition process is conducted on the blades while they are assembled as a blade assembly on a compressor or turbine rotor disc (53).

2. A method as claimed in Claim 1 in which the deposition process comprises producing a binding coat (81) on tips of bodies of the blades by electrolytic or electroless deposition, the binding coat comprising MCrAlY where M is one or more of iron, nickel and cobalt, anchoring to the binding coat with an achoring coat (82) coarse particles (83) of an abrasive material by composite electrolytic or electroless deposition from a bath of plating solution having the abrasive particles suspended therein, and then plating an infill (84) around the abrasive particles.

3. A method as claimed in Claim 2 in which the anchoring coat (82) is cobalt or nickel.

4. A method as claimed in Claim 2 in which the anchoring coat (82) is MCrAlY where M is Ni or Co or Fe or two or all of these metals.

5. A method as claimed in Claim 3 or Claim 4 in which the thickness of the anchoring coat (82) is less than 30 µm.

6. A method as claimed in any one of claims 2 to 5 in which the infill (84) comprises MCrAlY where M is Ni or Co or Fe or two or all of these metals.

7. A method as claimed in any of the Claims 2 to 6 in which deposition of the infill (84) is followed by a heat treatment step applied to the assembly to homogenise the binding coat (81), the anchoring coat (82) and the infill (84).

8. A method as claimed in any one of Claims 2 to 6 in which deposition of the infill (84) is followed by heat treatment from between ½ and 1 hour at 1090 plus or minus 10°C in vacuum or in 50-100 millibar partial pressure argon, and fast gas quenching.

9. A method as claimed in Claim 7 or Claim 8 in which the heat treatment is followed by an aluminizing step to aluminize the blade tips.

10. A method as claimed in any of the preceding claims in which at least part of the deposition is accompanied by vibration of the assembly, preferably in a vertical direction.

## Patentansprüche

1. Verfahren zum Erzeugen von abrasiven Kompressor- oder Turbinen-Rotorschaufelspitzen durch elektrolytisches oder stromloses Auftragen, dadurch gekennzeichnet, daß mindestens ein Teil des Auftrages auf die Schaufeln erfolgt, während diese als Schaufelgruppe auf einer Kompressor- oder Turbinen-Rotorscheibe (53) montiert sind.

2. Verfahren nach Anspruch 1, bei dem im Zuge des Auftragprozesses ein MCrAlY aufweisender Bindeüberzug (81) auf den Spitzen der Schaufelkörper durch elektrolytisches oder stromloses Auftragen erzeugt wird, wobei M Eisen und/oder Nickel und/oder Kobalt ist, mit dem Bindeüberzug mittels eines Verankerungsüberzuges (82) grobe Teilchen (83) aus einem abrasiven Werkstoff durch elektrolytisches oder stromloses Verbundauftragen aus einem Bad einer Beschichtungslösung, in welcher die abrasiven Teilchen suspendiert sind, verankert werden, und dann um die abrasiven Teilchen herum eine Füllung (84) aufgebracht wird.

3. Verfahren nach Anspruch 2, bei dem der Verankerungsüberzug (82) aus Kobalt oder Nickel besteht.

4. Verfahren nach Anspruch 2, bei dem der Verankerungsüberzug (82) aus MCrAlY besteht, wobei M Nickel und/oder Kobalt und/oder Eisen ist.

5. Verfahren nach Anspruch 3 oder Anspruch 4, bei dem die Dicke des Verankerungsüberzuges (82) kleiner als 30 µm ist.

6. Verfahren nach einem der Ansprüche 2 bis 5, bei dem die Füllung(84) MCrAlY aufweist, wobei M Nickel und/oder Kobalt und/oder Eisen ist.

7. Verfahren nach einem der Ansprüche 2 bis 6, bei dem auf das Aufbringen der Füllung (84) ein Wärmebehandlungsschritt folgt, dem die Baugruppe unterzogen wird, um den Bindeüberzug (81), den Verankerungsüberzug (82) und die Füllung (84) zu homogenisieren.

8. Verfahren nach einem der Ansprüche 2 bis 6, bei dem auf das Aufbringen der Füllung (84) eine Wärmebehandlung von ½ bis einer Stunde bei 1090 ± 10 °C in Vakuum oder in Argon mit einem Partialdruck von 50 bis 100 mbar, sowie ein rasches Abschrecken mit Gas folgen.

9. Verfahren nach Anspruch 7 oder Anspruch 8, bei dem auf die Wärmebehandlung ein Aluminierungsschritt folgt, um die Schaufelspitzen zu aluminieren.

10. Verfahren nach einem der vorhergehenden Ansprüche, bei dem während mindestens eines Teils des Auftragens die Baugruppe in vorzugsweise vertikaler Richtung in Vibration versetzt wird.

## Revendications

1. Procédé de production d'extrémités abrasives sur des ailettes de rotor de turbine ou de compresseur par dépôt électrolytique ou sans courant, caractérisé en ce qu'au moins une partie du processus de dépôt est effectuée sur les ailettes lorsqu'elles sont assemblées en un montage d'ailettes sur un rotor (53) de compresseur ou de turbine.

2. Procédé suivant la revendication 1, dans lequel le processus de dépôt comprend la production d'une couche liante (81) sur des extrémités de corps des ailettes par dépôt électrolytique ou sans courant, la couche liante comportant du MCrAlY, où M est un ou plusieurs des éléments suivants : fer, nickel et cobalt, l'ancrage à la couche liante au moyen d'une couche d'ancrage (82) de particules grossières (83) d'une matière abrasive par dépôt sans courant ou électrolytique mixte à partir d'un bain d'une solution de plaquage contenant en suspension les particules abrasives, et ensuite le plaquage d'une matière de remplissage (84) autour des particules abrasives.

3. Procédé suivant la revendication 2, dans lequel la couche d'ancrage (82) est du cobalt ou du nickel.

4. Procédé suivant la revendication 2, dans lequel la couche d'ancrage (82) est du MCrAlY, où M est du Ni ou du Co ou du Fe ou deux de ces métaux ou tous ceux-ci.

5. Procédé suivant la revendication 3 ou 4, dans lequel l'épaisseur de la couche d'ancrage (82) est inférieure à 30 µm.

6. Procédé suivant l'une quelconque des revendications 2 à 5, dans lequel la matière de remplissage (84) comporte du MCrAlY où M est du Ni ou du Co ou du Fe ou deux de ces métaux ou tous ceux-ci.

7. Procédé suivant l'une quelconque des revendications 2 à 6, dans lequel le dépôt de la matière de remplissage (84) est suivi d'une étape de traitement thermique appliquée au montage pour homogénéiser la couche liante (81), la couche d'ancrage (82) et la matière de remplissage (84).

8. Procédé suivant l'une quelconque des revendications 2 à 6, dans lequel le dépôt de la matière de remplissage (84) est suivi d'un traitement thermique d'une durée comprise entre ½ et 1 heure à 1090°C plus ou moins 10°C sous vide ou sous une pression partielle d'argon de 50-100 millibars et d'une trempe rapide par du gaz.

9. Procédé suivant la revendication 7 ou 8, dans lequel le traitement thermique est suivi d'une étape d'aluminisation pour recouvrir d'aluminium les extrémités des ailettes.

10. Procédé suivant l'une quelconque des revendications précédentes, dans lequel au moins une partie du dépôt est accompagnée par la mise en vibration du montage, de préférence dans une direction verticale.
